

Sept. 12, 1939.

C. A. WEBB

2,172,425

RUBBER PLAYING BALL

Filed May 10, 1937

*Fig.1.*



*Fig. 2.*



Inventor

*Charles A. Webb,*

*By Harry Booth Holman & Dix  
his Attorney*

Patented Sept. 12, 1939

2,172,425

# UNITED STATES PATENT OFFICE

2,172,425

## RUBBER PLAYING BALL

Charles A. Webb, Lebanon, Pa., assignor to C. E. Webb Co., Lebanon, Pa., a copartnership composed of C. B. Webb and Grace I. Webb

Application May 10, 1937, Serial No. 141,810

10 Claims. (CL. 273—65)

The present invention relates to rubber playing balls and particularly to rubber athletic balls, such as footballs, volley balls, soccer balls, basket balls and the like and the invention aims generally to improve such articles.

Athletic balls of the type referred to above usually comprise a leather cover and an inflatable rubber bladder therefor, and such balls have become standard balls in professional, varsity and scholastic athletics. Such balls are relatively inexpensive, particularly for elementary school games and practice work, and there is a decided demand for an inexpensive rubber practice ball, simulating substantially the leather covered ball in size, weight, feel and bounce.

The problem of making an inflated rubber playing ball to simulate a leather covered athletic ball in size, weight and appearance is not difficult and involves merely the making of an ordinary inflated rubber ball of proper size and thickness to conform to the standard sizes and weights of corresponding leather covered athletic balls. Such balls, however, have not heretofore corresponded to the leather covered athletic balls in resilience or bounce, as the rubber compounds commonly used in the manufacture of inflated playing balls provide a too lively ball, particularly when inflated to an extent to have a feel or handle corresponding to a similar standard leather covered ball. This is particularly disadvantageous in connection with inflated rubber soccer balls, foot balls and basket balls, as the lively or highly bouncing ball leads to a very difficult style of play than the less lively leather covered standard ball.

I have discovered that a compound containing rubber as a principal ingredient, combined with stiffening ingredients which will increase the tensile strength, lower the specific gravity of the compound as well as soften it for suitable molding under heat is highly satisfactory for the manufacture of hollow inflated rubber balls having the characteristics of appearance, feel, resilience, stiffness and weight of standard leather covered balls of the types above described.

While the invention is not restricted to the manufacture of any particular type of inflated athletic ball, I have illustrated in the accompanying drawing a suitable construction of basket ball which may be made according to the invention.

In the drawing—

Fig. 1 is a plan view of the ball; and

Fig. 2 is a detail sectional view thereof.

According to the invention, the ball 10 may be of any desired size and shape to correspond to

a standard leather covered athletic ball, as for example, a foot ball, soccer ball, volley ball or basket ball, the latter being selected as an illustrative embodiment. The ball advantageously is formed of pre-shaped halves cemented together along a median line, and thereafter vulcanized in a mold as is usual. Preferably the ball is inflated through a self-closing valve 11 of suitable type and construction so that it may be inflated with air to a proper pressure, this being preferable to the so-called gas filled balls wherein the pressure cannot be accurately regulated. Preferably the surfaces of the curing molds are engraved to produce irregular dimpled designs of convex form on the surface of the ball, as at 12, to imitate tanned pigskin or other leather used in the manufacture of standard leather covered athletic balls. Also the molds are constructed to mold into the body of the ball grooves 13, imitating seams of a leather covered ball and imitation lacing 14, and imitation stitching 15.

In order that the inflated rubber balls may possess a resilience and stiffness substantially corresponding to the resilience and stiffness of corresponding standard leather covered balls, I preferably form the balls of a compound composed of rubber, a stiffening and deadening ingredient, preferably a mineral powder, such as carbon black or magnesium carbonate, and thermo-plastics, such as wax, glue, shellac or paraffin to soften the surface of the rubber by the curing heat so that the leather design may be embossed therein, combined with usual curing agents.

Preferably the compound may include the following—

|                       | Pounds   |
|-----------------------|----------|
| Rubber                | 100      |
| Stiffening ingredient | 30-80    |
| A thermo-plasticiser  | 10-40 40 |

and usual curing agents.

The rubber ingredients may be pure rubber or partly pure and partly reclaim, as is well understood. To this a substantial amount of stiffening ingredient is added to stiffen the rubber and increase the tensile strength of the compounds. A mineral, such as carbon black and magnesia carbonate, have been found highly suitable for this purpose and either materially stiffens and increases the tensile strength of the compound when mixed with the rubber.

Such compound could not be molded readily, as for example, in vulcanizing molds, where an accurate ornamental design, such as imitation

leather, is to be produced on the surface of the ball. Accordingly, I add to the compound a suitable thermo-plasticiser such as wax, paraffin, glue or shellac which will act to soften the compound during the vulcanization to permit the compound to flow to the shape of the mold, but which will act to stiffen the compound upon cooling. This thermo-plasticiser also functions to decrease the resilience of the compound.

10 In the manufacture of certain athletic rubber balls it is desirable to lower the specific gravity of the compound so as to more accurately simulate the standard leather cover ball in weight and feel. Accordingly, the stiffening ingredient may include in the above stated example, from 10 to 40 pounds of a lightening stiffener, for example cellulose, such as wood flour, cotton flock, rayon flock or the like. Such cellulose is highly advantageous as it does not soften the cured compound but on the other hand increases its stiffness.

15 It will be noted that the various ingredients compounded with the rubber, excepting the usual curing agents, add to the stiffness of the compound, and therefore decrease the resiliency of the ball, when inflated. In addition to these stiffening properties, the carbon black or magnesium carbonate materially increases the tensile strength of the ball, and the cellulose lowers the specific 20 gravity of the compound so that the ball may be of substantial thickness to give the desired feel to the ball. Similarly the thermo-plasticiser adds stiffness in the finally cured article, but when subjected to the heat of vulcanization, softens the compound and permits it to flow to the contour 25 of the molds. It is thus possible to mold the compound during vulcanization to produce a lightly dimpled surface having a realistic appearance 30 of leather.

35 40 A hollow playing ball of any of the above named types and of proper size, shape and weight made of rubber and a compound as disclosed above, will correspond when properly inflated substantially in resilience, stiffness and feel to the more expensive corresponding standard leather covered 45 balls of the usual bladder inflated design and may be satisfactorily used in practice by elementary schools, permitting a style of play not differing radically from the style of play required when using the standard leather covered 50 balls.

55 I am aware that heretofore some of the ingredients mentioned above have been compounded with rubber for the manufacture of other non-analogous articles. However, so far as I 60 am aware neither these nor similar ingredients have ever been included in a rubber compound for the manufacture of hollow inflated playing balls to impart to the balls the highly desirable properties achieved by my invention.

65 It will be apparent to those skilled in the art that proportions and amounts of ingredients may be varied considerably to obtain the desired characteristics of the playing ball, and that the invention is highly useful and desirable in the manufacture of inflated rubber playing balls other than those simulating leather covered bladder-inflated athletic balls. Accordingly, the invention is not to be restricted to the details illustrated and described, and the scope of the invention is more fully defined by the appended claims.

I claim:

70 75 1. An inflated rubber playing ball formed of a vulcanized compound containing rubber and a

stiffening ingredient adapted to stiffen the compound and increase the tensile strength, and an ingredient capable of softening the compound to render it moldable under heat of vulcanization but capable of increasing the stiffness of the compound upon cooling.

2. An inflated rubber playing ball formed of a vulcanized compound containing rubber and a stiffening ingredient adapted to stiffen the compound and increase the tensile strength, and an ingredient selected from the group consisting of wax, glue, shellac and paraffin capable of softening the compound to render it moldable under heat of vulcanization but capable of increasing the stiffness of the compound upon cooling. 15

3. A hollow rubber sports ball having a dimpled surface resembling tanned leather, said ball being formed of a compound containing rubber, stiffening ingredients adapted to increase the tensile strength of the compound and a thermo-plasticiser to soften the compound under heat, to permit the ornamentation of said surface. 20

4. A hollow rubber sports ball having a dimpled surface resembling tanned leather, said ball being formed of a compound containing rubber, a stiffening ingredient and a thermo-plasticiser adapted to soften the compound under heat to permit the ornamentation of said surface. 25

5. An inflated rubber playing ball formed of a vulcanized compound of rubber, a stiffening ingredient selected from the group consisting of carbon black and magnesium carbonate, to increase the stiffness and tensile strength of the compound and a thermo-plastic ingredient selected from the group consisting of wax, glue, 30 shellac and paraffin to soften the compound under vulcanizing heat to permit molding, but upon cooling to stiffen and decrease the resilience of the compound.

6. An inflated rubber playing ball formed of a vulcanized compound of rubber, a stiffening ingredient selected from the group consisting of carbon black and magnesium carbonate, to increase the stiffness and tensile strength of the compound, a cellulose ingredient to lower the specific 45 gravity of the compound and a thermo-plastic ingredient selected from the group consisting of wax, glue, shellac and paraffin to soften the compound under vulcanizing heat to permit molding, but upon cooling to stiffen and decrease 50 the resilience of the compound.

7. An inflated rubber playing ball formed of a vulcanized compound containing rubber and a stiffening ingredient in substantial amounts, 30 to 80 per cent by weight, of the rubber content, 55 adapted to stiffen the compound and increase the tensile strength, and an ingredient capable of softening the compound to render it moldable under heat of vulcanization but capable of increasing the stiffness of the compound upon 60 cooling.

8. An air inflated rubber playing ball of desired appearance and shape corresponding to a leather covered athletic ball of desired type, said ball composed of a cured compound of rubber, a stiffening ingredient to lower the resiliency of the ball to substantially correspond to the resiliency of such leather covered athletic balls and an ingredient capable of softening the compound to render it moldable under heat of vulcanization but capable of increasing the stiffness of the compound upon cooling. 70

9. A hollow rubber sports ball having a dimpled surface resembling tanned leather, said ball being formed of a compound containing rubber, a 75

stiffening ingredient including a cellulose material adapted to lower the specific gravity of the compound and a thermo-plasticiser adapted to soften the compound under heat to permit the ornamentation of said surface.

5 10. A hollow rubber sports ball having a dimpled surface resembling tanned leather, said ball being formed of a compound containing

rubber, a stiffening ingredient including a material selected from the group comprising wood flour, cotton flock or rayon flock adapted to lower the specific gravity of the compound, and a thermo-plasticiser adapted to soften the compound under heat to permit the ornamentation of said surface.

CHARLES A. WEBB.